

## UNITED STATES PATENT OFFICE

2,136,757

AFTER-TREATMENT OF DYEINGS ON CEL-  
LULOSIC FIBERSHans Roos, Leverkusen-I. G.-Werk, Germany, as-  
signor to General Aniline Works, Inc., New  
York, N. Y., a corporation of DelawareNo Drawing. Application June 5, 1935, Serial  
No. 25,182. In Germany June 29, 1934

16 Claims. (Cl. 8—46)

This invention relates to a process for the improvement of the fastness to washing of dyeings on cellulosic fibers with substantive dyestuffs and to the improved dyeings obtained by this process.

In accordance with the present invention the fastness to washing of dyeings on cellulosic fibers with substantive dyestuffs containing at least once the grouping

10



wherein R and R' stand for aromatic radicals, is improved by aftertreating the same in the manner known per se with diazo compounds of the aromatic series. For the purpose of the present invention there come into consideration quite generally those bases as are used in the manufacture of ice colors, i. e. bases containing no substituents inducing solubility in water, especially of the benzene series, such as anisidine, para-nitro-ortho-anisidine and, first of all, nitranilines. The process is carried out by introducing the fiber dyed with a dyestuff of the kind above identified into a diazo solution prepared in the usual manner and in which the mineral acid has been neutralized, for example, by adding sodium acetate, for about half an hour at room temperature, rinsing the fiber, soaping the same in a boiling bath, again rinsing and drying. By this aftertreatment the fastness to washing is considerably improved; further, the dyeings possess a better fastness to light than dyeings with analogously constituted dyestuffs produced by other methods, and, moreover, they may have a very good dischargeability with a neutral or alkaline reacting discharge paste.

The following examples will illustrate the invention without, however, restricting it thereto:—

## Example 1

Cotton is dyed from a Glauber's salt-soda-bath with the reduced dyestuff from one molecular proportion of para-aminobenzoyl-p-aminophenylurea-disulfonic acid and 2 molecular proportions of 1-(meta-nitrophenyl)-5-pyrazolone-

3-carboxylic acid, said dyestuff corresponding in its free state to the following formula:—



10 grams of the dyed cotton are introduced for about half an hour into a bath containing 0.3 gram of diazotized para-nitraniline, said bath being prepared by diazotizing in the usual manner para-nitraniline with hydrochloric acid and sodium nitrite and neutralizing the mineral acid by the addition of sodium acetate. By this aftertreatment a reddish-yellow shade is obtained of very good fastness to light and dischargeability in 25 the neutral and alkaline processes.

## Example 2

Cotton is dyed from a Glauber's salt-soda bath with the dyestuff obtainable by coupling diazotized para-nitrobenzoyl-p-phenylenediamine with 1-(meta-nitrophenyl)-5-pyrazolone-3-carboxylic acid, reducing the nitro group to the amino group, diazotizing, coupling with 1-(meta-nitrophenyl)-5-pyrazolone-3-carboxylic acid and reducing the 35 nitro group, said dyestuff corresponding to the following formula:—



The orange dyeing thus obtained is aftertreated with para-nitraniline and yields a clear yellow-orange shade exhibiting properties similar to those of the aftertreated dyeing of Example 1.

5

**Example 3**

Cotton is dyed from a Glauber's salt-soda-bath with a dyestuff obtainable by diazotizing acetyl-10 para-phenylene diamine, coupling with salicylic acid, saponifying the acetylaminogroup, condensing with para-nitro-benzoylchloride, reducing the nitro group to the amino group, diazotizing and coupling with 1-(meta-aminophenyl)-5-15 pyrazolone-3-carboxylic acid, which dyestuff corresponds to the following formula:—



40 The yellow dyeing thus obtained is aftertreated with diazotized para-nitraniline. It is of a somewhat more greenish shade than that of Example 1, exhibits a better fastness to light and has otherwise similar properties.

45 When using in the above example instead of the 1-(meta-aminophenyl)-5-pyrazolone-3-carboxylic acid the 1-(para-aminophenyl)-5-pyrazolone-3-carboxylic acid and aftertreating in the usual manner with diazotized para-nitraniline, brownish-yellow shades are obtained of an especially good neutral or alkaline dischargeability.

50 When using in the above example for the after-

nitro group, which dyestuff corresponds to the following formula:—



The yellowish orange dyeing is aftertreated with diazotized para-nitraniline. Thus an orange dyeing is obtained exhibiting properties similar to those of the aftertreated dyeing of Example 2.

**Example 5**

Cotton is dyed in the usual manner from a Glauber's salt-soda-bath with the dyestuff obtained by diazotizing ortho-amino-benzoic acid and coupling with para-aminobenzoyl-2-amino-5-naphthol-7-sulfonic acid, diazotizing and coupling with 1-(meta-aminodiphenyl)-5-pyrazolone-3-carboxylic acid, which dyestuff corresponds to the following formula:—



40 An orange dyeing is thus obtained which becomes somewhat more yellowish after the aftertreatment with diazotized para-nitraniline. It is distinguished by an excellent clarity and fastness to light combined with a good neutral and alkaline dischargeability.

**Example 6**

Cotton is dyed in the usual manner from a Glauber's salt-soda-bath with the dyestuff from diazotized meta-aminobenzoyl-dehydro-thiotoluidine sulfonic acid and 1-(meta-aminophenyl)-5-pyrazolone-3-carboxylic acid of the formula:—



60 treatment instead of the diazotized para-nitraniline the 4-nitro-ortho-anisidine or 5-nitro-ortho-anisidine ( $\text{OCH}_3=1$ ), somewhat more reddish shades are obtained.

65

**Example 4**

70 Viscose silk is dyed from a Glauber's salt-soda-bath with the dyestuff obtained by coupling one molecular proportion of tetrazotized para-aminobenzyl-para-phenylene-diamine, one molecular proportion of ortho-cresotinic acid and one molecular proportion of 1-(meta-nitrophenyl)-5-pyrazolone-3-carboxylic acid, and reducing the

75 I claim:—

1. The process which comprises aftertreating cellulosic fibers which have been dyed with a substantive dyestuff containing at least once the grouping



65

70

75

wherein R and R' stand for aromatic radicals, with a diazo compound of an aromatic amine free from a group inducing solubility in water.

2. The process as claimed in claim 1, in which the fibers are aftertreated with a diazotized nitraniline.

3. The process as claimed in claim 1, in which the fibers are aftertreated with diazotized para-nitraniline.

10 4. The process which comprises aftertreating cellulosic fibers which have been dyed with a substantive dyestuff of the formula:—



20 wherein R and R' stand for aromatic radicals and R<sub>2</sub> stands for an aromatic radical which may contain an azo group, with a diazo compound of an aromatic amine free from a group inducing solubility in water.

25 5. The process as claimed in claim 4, in which the fibers are aftertreated with a diazotized nitraniline.

6. The process as claimed in claim 4, in which the fibers are aftertreated with diazotized para-nitraniline.

30 7. The process which comprises aftertreating cellulosic fibers which have been dyed with the dyestuff of the formula:—



with diazotized para-nitraniline.

50 8. The process which comprises aftertreating cellulosic fibers which have been dyed with the dyestuff of the formula:—



65 with diazotized para-nitraniline.

9. Cellulosic fibers dyed with a dyestuff containing at least once the grouping:



75 wherein R and R' stand for aromatic radicals

and R'' stands for an aryl radical free from a group inducing solubility in water.

10. Cellulosic fibers dyed with a dyestuff containing at least once the grouping:



wherein R and R' stand for aromatic radicals.

11. Cellulosic fibers dyed with a dyestuff containing at least once the grouping:



wherein R and R' stand for aromatic radicals.

12. Cellulosic fibers dyed with a dyestuff of the formula:



wherein R and R' stand for aromatic radicals, R'' stands for an aryl radical free from a group inducing solubility in water, and R''' stands for



an aromatic radical which may contain an azo group.

13. Cellulosic fibers dyed with a dyestuff of the formula:



wherein R and R' stand for aromatic radicals and R''' stands for an aryl radical which may contain an azo group.

14. Cellulosic fibers dyed with a dyestuff of the formula:



wherein R and R' stand for aromatic radicals and R''' stands for an aryl radical which may contain an azo group.

15. Cellulosic fibers dyed with the dyestuff of the formula:



**16. Cellulosic fibers dyed with the dyestuff of the formula:**



**HANS ROOS.**